

1

3,332,756

**GASOLINE MOTOR FUEL COMPOSITION**  
John F. Deffner, Glenshaw, Pa., assignor to Gulf Research & Development Company, a corporation of Delaware  
No Drawing. Filed June 13, 1963, Ser. No. 287,488  
4 Claims. (Cl. 44—69)

This invention relates to fuels and more particularly to leaded gasolines for high-compression, spark ignition engines.

It has long been recognized that for greater economy with respect to fuel requirement and greater efficiency in the operation of a gasoline-powered, spark ignition engine, high compression ratios are desired. As a result, several automobile manufacturers have increased the compression ratios of their spark ignition engines to 8.5:1 and even as high as 10.5:1, the future trend of the automotive industry indicating that substantially all engines will be operating at such high or higher compression ratios in the foreseeable future. In order to obtain smooth engine operation at these high compression ratios under various driving conditions it is necessary to employ a fuel having high octane numbers as determined by both the motor method (ASTM: D357-53) and the research method (ASTM: D908-55).

Smooth operation at high speeds under open-road conditions in modern high-compression engines usually requires a fuel having a motor octane number of at least about 85. Smooth operation in the same engines at lower speeds under city driving conditions where frequent accelerations are encountered usually requires a fuel having a research octane number of at least about 95. An optimum fuel for present day use is thus one which has a research octane number of at least about 95 and a sensitivity of about 8 to 12. By "sensitivity," I intend to indicate the spread or differential between the octane numbers as determined by the motor method and the research method. Of course, if fuels are available whose motor and research octane numbers coincide at levels of 95 or more, the sensitivity of such fuels can be in the order of 1 to 2 or less and still result in desirable fuels for use in high-compression engines under both low-speed and high-speed operation.

In order to obtain fuels having both high motor and high research octane numbers the petroleum industry has developed numerous petroleum hydrocarbon conversion processes among which may be mentioned cracking, alkylation, aromatization, cyclization, isomerization, hydrogenation, dehydrogenation, hydroisomerization, polymerization, hydrodesulfurization, reforming, hydroforming, polyforming, "Platforming" and combinations of two or more of such processes. These processes produce hydrocarbons boiling in the gasoline boiling range which have engine performance characteristics markedly superior to the charge stock and to comparable boiling hydrocarbons found in straight-run gasolines. In general, straight-run gasolines are more paraffinic and less olefinic and aromatic than gasolines obtained, for example, by a cracking process. Straight-run gasolines, *per se*, even when fortified with tetraethyl lead generally do not give the high motor and research octane numbers required for smooth performance in present day engines. This invention is concerned primarily, therefore, with fuels or a blend of fuels obtained by one or more of the above-mentioned hydrocarbon conversion processes. However, a small amount of straight-run gasoline, in some instances, may be blended with the fuels obtained by a conversion process.

To improve still further the octane ratings of the fuels obtained by the various conversion processes, the petroleum industry, in most instances, has resorted to the use of various anti-knock agents among which is tetraethyl

2

lead. While the addition of tetraethyl lead to gasolines obtained by one or more conversion processes improves their motor and research octane numbers, the resulting fuels have certain disadvantages arising from the presence of the lead. One of the chief objections to the use of gasolines containing tetraethyl lead, i.e., leaded gasolines, arises from the tendency of such fuels upon being burned to form decomposition products of tetraethyl lead, a portion of which products are deposited on the walls of the combustion chambers of the engine and on the electrodes and insulators of the spark plugs, thus reducing the efficiency of the engine and offsetting to some extent the increased efficiency obtained by using an engine having a high compression ratio.

In an attempt to overcome the detrimental effect of the deposits of tetraethyl lead decomposition products in an engine, various scavenging agents have been added to the fuel to change the form of the tetraethyl lead decomposition products to those which are more volatile and thus less likely to be deposited within the engine. For example, various volatile alkyl halides such as ethylene dibromide and/or ethylene dichloride have been used with tetraethyl lead to produce the corresponding halides of lead which are more volatile than the oxides. The volatile alkyl halides, however, have not completely overcome the deposition of the decomposition products. The decomposition products comprise various salts including the oxides, sulfates, bromides and chlorides of lead. These decomposition salts deposited within the combustion chamber of the engine have been found to alter adversely the engine operation. The adverse effect encountered as a result of the deposits of the decomposition salts is frequently evidenced by engine knocking. The knocking thus encountered is that associated with preignition of the fuel in the combustion chamber of a spark ignition engine. This knocking associated with preignition should not be confused with knocking due to explosive autoignition of the unburned portion of the fuel-air mixture to be traversed by the normal flame from the spark plug.

I have found that the decomposition salts deposited within the combustion chamber of a high-compression, spark ignition engine can be modified to reduce their tendency to promote or initiate preignition of the motor fuel in the engine by incorporating in the motor fuel a small amount of a metal carbonyl selected from the group consisting of molybdenum hexacarbonyl and tungsten hexacarbonyl. Thus, in accordance with the present invention an improved gasoline motor fuel composition comprises a major amount of a gasoline containing tetraethyl lead in an amount sufficient to produce a gasoline fuel composition having a motor octane number of at least about 85 and a research octane number of at least about 95, said gasoline fuel composition upon combustion normally tending to form deposits which induce preignition of the gasoline in the combustion chamber of a high-compression, spark ignition engine and a small amount, sufficient to substantially reduce such preignition, of a metal carbonyl, selected from the group consisting of molybdenum hexacarbonyl and tungsten hexacarbonyl.

The hexacarbonyls of molybdenum and tungsten are available commercially and thus their preparation, *per se*, constitutes no part of the present invention. They can readily be prepared, for example, by reacting a salt of the metal such as tungsten hexachloride with carbon monoxide and a reducing metal such as aluminum in the presence of a catalytic amount of a metal alkyl such as triethyl aluminum. The reaction is conducted at temperatures up to about 200° C. and at pressures up to about 5,000 pounds per square inch.

The amount of the hexacarbonyl of molybdenum or

tungsten employed depends upon the tetraethyl lead content of the fuel. For this reason, the amount is more significant and is more accurately expressed in terms of that amount which theoretically would be required if all of the lead introduced into the fuel in the form of tetraethyl lead were to be converted to lead molybdate or lead tungstate assuming 100 percent conversion. While improved results can be obtained in some instances with amounts corresponding to at least about 0.05 times that theoretically required to convert the lead to lead molybdate or lead tungstate, it is ordinarily preferred to use amounts above about 0.1 theory. Especially good results are obtained by using about 0.2 times the theoretical amount required. In general, I prefer to use an amount not more than about 0.3 times the theoretical amount required to convert all of the lead to lead molybdate or lead tungstate. Amounts greater than 0.3 times the theoretical amount can be employed, but for economic reasons, I prefer to use only the amount required to give the desired improvement. Amounts in the order of at least about 0.005 theory can be employed when another ignition control agent, such as an organo-phosphorus compound, is also present in amounts of 0.1 to 0.5 theory. The metal carbonyls at lower concentrations have less tendency to adversely affect the octane rating of the leaded gasoline in which they are incorporated. Therefore, I prefer to employ the least amount of metal carbonyl required to give the desired improvement within the range of about 0.05 to about 0.3 times that theoretically required to convert the lead to lead molybdate or lead tungstate. In view of the fact that the amount of tetraethyl lead in the gasoline varies from one fuel to another, it is difficult to state on a weight basis the amount of the hexacarbonyl compound based upon the weight of the gasoline. However, once knowing the amount of tetraethyl lead present in the gasoline, it is an easy matter to calculate the amount of the hexacarbonyl compound required on a weight basis. Most gasolines on the market today contain between about one and about three cubic centimeters of tetraethyl lead per gallon of gasoline. Based upon a gasoline having a gravity of about 54° API and containing about one cubic centimeter of tetraethyl lead, I have determined that the amount of molybdenum hexacarbonyl corresponding to 0.05 to 0.3 theory is about 0.002 to about 0.014 percent by weight based on the gasoline. To incorporate 0.05 to 0.3 theory of tungsten hexacarbonyl in the same gasoline would require about 0.003 to about 0.019 percent by weight based on the gasoline. If the gasoline contains 3 cubic centimeters of tetraethyl lead, then the molybdenum hexacarbonyl for 0.05 to 0.3 theory is about 0.007 to about 0.042 percent by weight. In this case, the tungsten hexacarbonyl would correspond to about 0.009 to about 0.056 percent by weight. Thus, the normally useful concentration range for a 54° API gasoline containing about 1 to about 3 cubic centimeters of tetraethyl lead is about 0.002 to about 0.06 percent. It will be understood, of course, that the optimum amount on a weight basis for molybdenum hexacarbonyl may not be the optimum amount for tungsten hexacarbonyl. One reason for this is that the effectiveness of the compounds may vary. Another quite obvious reason is that the molecular weight of tungsten hexacarbonyl (352) is greater than the molecular weight of molybdenum hexacarbonyl (264). In any event, the amount of the molybdenum hexacarbonyl or tungsten hexacarbonyl used is sufficient to modify the decomposition salts deposited within the combustion chamber of a high-compression, spark ignition engine to reduce their tendency to promote or initiate preignition of a gasoline containing tetraethyl lead and an ethylene halide in an amount normally tending upon combustion to form deposits which induce preignition of the gasoline in the combustion chamber of the engine.

The gasoline fuel composition to which the molybdenum hexacarbonyl or tungsten hexacarbonyl is added comprises

a mixture of hydrocarbons boiling in the gasoline boiling range having a motor octane number (leaded) of at least about 85 and a research octane number (leaded) of at least about 95. The mixture of hydrocarbons can be obtained by at least one of the petroleum conversion processes including cracking, alkylation, aromatization, cyclization, isomerization, hydrogenation, dehydrogenation, hydrosomerization, polymerization, hydrodesulfurization, reforming, hydroforming, polyforming, "Platforming," and combinations of two or more such processes, as well as by the Fischer-Tropsch and related processes. While current straight-run gasoline has octane numbers too low to qualify as the sole hydrocarbon component of gasoline fuel compositions within the scope of this invention, a small amount of straight-run gasoline can be blended with the hydrocarbon mixture obtained by one or more of the designated conversion processes provided the resulting mixture has a motor octane number (leaded) of at least about 85 and a research octane number (leaded) of at least about 95. A preferred gasoline fuel composition comprises a blend of hydrocarbons obtained by catalytic cracking, "Platforming" and alkylation processes.

In addition to the molybdenum or tungsten hexacarbonyl and tetraethyl lead, the gasoline fuel composition of my invention can contain other gasoline improvement agents including upper cylinder lubricants, corrosion and oxidation inhibitors, conventional alkyl halide lead scavenging agents, alcoholic anti-stalling agents, metal deactivators, dehazing agents, anti-rust additives, other ignition control agents, dyes and the like.

In a preferred embodiment of the invention, about 0.02 to about 0.1 theory of the metal hexacarbonyl is employed in conjunction with about 0.1 to about 0.5 theory of a phosphorus-containing ignition control agent. For example, about 0.02 to about 0.1 theory of tungsten or molybdenum hexacarbonyl is employed together with about 0.1 to about 0.5 theory of an organo-phosphorus compound such as tricresyl phosphate, cresyl diphenyl phosphate, methyl diphenyl phosphate, tri(n-butyl)phosphate, tri(butoxyethyl)phosphate, tributyl phosphite, trimethylphosphite, tributyl phosphine, and the like. When molybdenum or tungsten hexacarbonyl and tri(butoxyethyl)phosphate are used together, the molybdenum or tungsten hexacarbonyl is preferably employed in amounts corresponding to about 0.02 to about 0.1 theory and the tri(butoxyethyl)phosphate in an amount corresponding to about 0.1 to about 0.2 theory.

When an upper cylinder lubricant is employed it is generally used in an amount of from about 0.25 to about 0.75 percent by volume of the composition, e.g., 0.5 volume percent. This oil should be a light lubricating oil distillate, e.g., one having a viscosity at 100° F. of from about 50 to about 500 Saybolt Universal seconds, e.g., about 100 SUS. Although highly paraffinic lubricating distillates can be used, lubricating distillates obtained from Coastal or naphthenic type crude oils are preferred because of their superior solvent properties. The lubricating oil can be solvent-treated, acid-treated or otherwise refined.

When an oxidation inhibitor is desired any of the conventional inhibitors can be utilized. The alkylated phenols, e.g., 2,4,6-tri-tertiary-butylphenol, 2,6-di-tertiary-butyl-4-methylphenol, 2,2-bis(2-hydroxy-3-tertiary-butyl-5-methylphenyl)propane and bis(2-hydroxy-3-tertiary-butyl-5-methylphenyl)methane, because of their hydrocarbon-solubility and water-insolubility characteristics are preferred oxidation inhibitors. Such inhibitors when used are incorporated in the gasoline fuel composition in amounts of from about 0.001 to about 0.02 percent by weight of the composition, e.g., 0.007 weight percent.

Exemplary of other specific improvement agents which can be used are N,N'-disalicylidene-1:2-diaminopropane as a metal deactivator and the cocamine salt of diisooctyl acid orthophosphate as a rust inhibitor. The metal deactivator is generally used in small amounts of the order

of about 0.0003 to about 0.001 percent by weight based on the fuel composition. The rust inhibitor is generally used in small amounts of the order of about 0.002 to about 0.008 percent by weight based on the fuel composition.

The molybdenum and tungsten hexacarbonyls present no particular problem with respect to their addition to gasoline. While the hexacarbonyl can be added directly to the gasoline, one convenient method of adding it to the fuel is to form a concentrate thereof with a liquid solvent and thereafter adding the concentrate to the fuel. Any solvent which does not adversely affect the desirable properties of the fuel can be used. Suitable solvents include mineral oil, gasoline, naphtha, Stoddard solvent, mineral spirits, benzene, heptane, kerosene, toluene, ethyl alcohol, isopropyl alcohol, isoctyl alcohol, decyl alcohol, methylal, acetal, propylal and isopropylal, tetraethoxy propane, dimethyl acetal of isoctyl aldehyde, ethyl ether, cyclohexanol, acetone, an alkoxyalkanol, or the like. The concentrate, of course, can contain other conventional gasoline improvement agents, such as anti-oxidants, typical anti-stalling agents, anti-knock agents, a metal deactivator, an upper cylinder lubricant, an alkyl halide lead scavenging agent, a dehazing agent, anti-rust additives, other ignition control agents, dyes and the like. Since the amount of hexacarbonyl employed depends upon the amount of the tetraethyl lead present, this method of adding the compound to the gasoline serves as a convenient way of adding the correct amount of hexacarbonyl and tetraethyl lead simultaneously. Thus, a gasoline-benefiting concentrate can be made by admixing tetraethyl lead or commercially available mixtures of tetraethyl lead and a halide of ethylene and a solvent such as benzene or toluene with the molybdenum or tungsten hexacarbonyl wherein the hexacarbonyl is present in an amount between about 0.05 and about 0.3 times the theoretical amount required to convert the lead of the tetraethyl lead to lead molybdate or lead tungstate.

One convenient method of preparing a gasoline-benefiting concentrate is to start with a commercially available product comprising tetraethyl lead and the halides of ethylene. One such commercially available product consists of about 61.5 percent by weight of tetraethyl lead, about 17.9 percent by weight of ethylene dibromide, about 18.8 percent by weight of ethylene dichloride and about 1.8 percent by weight of kerosene. This commercially available product has a specific gravity of 1.587 at 20° C.

A typical gasoline-benefiting concentrate wherein the molybdenum hexacarbonyl is present in an amount corresponding to 0.2 times the theoretical amount required to convert the lead to lead molybdate is prepared by incorporating 5.06 cubic centimeters of the commercially available product designated hereinabove in a toluene or benzene solution containing 0.81 grams of molybdenum hexacarbonyl. 5.06 cubic centimeters of the commercially available product contains 3 cubic centimeters of tetraethyl lead.

The amount of the gasoline-benefiting concentrate added to gasoline will vary depending upon the octane improvement desired. Ordinarily, however, the concentrate is added in an amount sufficient to incorporate between about one and about three cubic centimeters of tetraethyl lead in a gallon of gasoline.

The gasoline compositions of this invention and their preparation are illustrated in detail by the following specific examples.

#### EXAMPLE I

A gasoline composition having excellent preignition characteristics is prepared by incorporating 0.813 grams of molybdenum hexacarbonyl in a gallon of the base gasoline (approximately 0.028 weight percent). The base gasoline is a blended gasoline made up of catalytically cracked gasoline, alkylate and "Platformate." The base

70  
75

gasoline contains about 3 cubic centimeters (4.94 grams) of tetraethyl lead per gallon of gasoline. In addition, the base gasoline contains as an oxidation inhibitor 2,6-di-tertiary-butyl-4-methylphenol (30 lbs./1000 bbls.) and as a metal deactivator N,N'-disalicylidene-1:2-diaminopropane (1 lb./1000 bbls.). The molybdenum hexacarbonyl thus comprises about 0.2 times the theoretical amount required to convert the lead of the tetraethyl lead to lead molybdate.

#### EXAMPLE II

Another composition is prepared in the manner of the foregoing Example I by incorporating 1.083 grams of tungsten hexacarbonyl in a gallon of the base gasoline (approximately 0.038 weight percent). The tungsten hexacarbonyl thus comprises about 0.2 times the theoretical amount required to convert the lead to lead tungstate.

Typical properties of the base gasoline and the base gasoline containing 0.2 theory of molybdenum hexacarbonyl and tungsten hexacarbonyl are as follows:

|    | Base Gasoline                                      | Base Gasoline plus 0.2 Theory Molybdenum Hexacarbonyl | Base Gasoline plus 0.2 Theory Tungsten Hexacarbonyl |
|----|----------------------------------------------------|-------------------------------------------------------|-----------------------------------------------------|
| 25 |                                                    |                                                       |                                                     |
| 30 | Gravity, ° API.....                                | 55.4                                                  | 55.4                                                |
|    | Sp. Gr., 60°/60° F.....                            | 0.7571                                                | 0.7571                                              |
|    | Sulfur, L, Percent.....                            | 0.040                                                 | 0.039                                               |
|    | Copper Strip Test, 122° F., 3 hrs.....             | 1                                                     | 1                                                   |
|    | Copper Dish Gum, mg./100 ml. (ASTM: D910-53T)..... | 20                                                    | 15                                                  |
|    | Existent Gum, mg./100 ml.....                      | 2                                                     | 5                                                   |
|    | Oxidation Stability, min.....                      | 1,064                                                 | 1,193                                               |
|    | Bromine No.....                                    | 29.7                                                  | 29.3                                                |
| 35 | Knock Rating:                                      |                                                       |                                                     |
|    | Motor Method.....                                  | 88.9                                                  | 87.7                                                |
|    | Research Method.....                               | 100.7                                                 | 99.8                                                |
|    | TEL, ml./gal.....                                  | 30.03                                                 | 3.12                                                |
|    | Vapor Pressure Reid, lb.....                       | 6.0                                                   | 6.0                                                 |
| 40 | Distillation, Gasoline:                            |                                                       |                                                     |
|    | Over Point, ° F.....                               | 108                                                   | 110                                                 |
|    | End Point, ° F.....                                | 381                                                   | 380                                                 |
|    | 10% Evap. at ° F.....                              | 165                                                   | 154                                                 |
|    | 50% Evap. at ° F.....                              | 253                                                   | 244                                                 |
|    | 90% Evap. at ° F.....                              | 323                                                   | 321                                                 |
|    | Recovery.....                                      | 98.2                                                  | 98.0                                                |
| 45 |                                                    | 97.2                                                  |                                                     |
|    | Residue.....                                       | 0.8                                                   | 0.8                                                 |
| 50 |                                                    | 1.0                                                   |                                                     |

#### EXAMPLE III

Another composition is prepared in the manner of the foregoing Example I by incorporating 0.406 grams of molybdenum hexacarbonyl in a gallon of base gasoline (approximately 0.014 weight percent). The molybdenum hexacarbonyl thus comprises about 0.1 times the theoretical amount required to convert the lead to lead molybdate.

#### EXAMPLE IV

An additional composition is prepared in the manner of the foregoing Example I by incorporating 0.203 grams of molybdenum hexacarbonyl in a gallon of gasoline. The molybdenum hexacarbonyl thus comprises about 0.05 times the theoretical amount required to convert the lead to lead molybdate.

#### EXAMPLE V

An additional gasoline composition having improved preignition characteristics combined with good upper-cylinder lubrication is prepared by adding a lubricating oil distillate to the base gasoline and then incorporating in the oil-containing gasoline fuel composition 0.813 grams of molybdenum hexacarbonyl per gallon of gasoline fuel composition (approximately 0.028 weight percent). The molybdenum hexacarbonyl thus comprises about 0.2 times the theoretical amount required to convert the lead to lead molybdate. The base gasoline used prior to the addition of the additives is the same

as that used in Examples I through IV. The oil, a light Coastal type (Texas) lubricating distillate oil, is added to the base gasoline in the amount of 0.5 percent by volume (approximately 0.6 percent by weight) in order to form the oil-containing gasoline fuel composition. Typical properties of the lubricating distillate oil are as follows:

|                                     |       |    |
|-------------------------------------|-------|----|
| Gravity, ° API                      | 24.5  | 10 |
| Lbs./gal., 60° F.                   | 7.55  |    |
| Viscosity, SUS:                     |       |    |
| 70° F.                              | 235   |    |
| 100° F.                             | 106.0 | 15 |
| 130° F.                             | 63.9  |    |
| 210° F.                             | 38.3  |    |
| Viscosity Index                     | 16    |    |
| Flash, P-M: ° F.                    | 315   |    |
| Flash, OC: ° F.                     | 320   |    |
| Fire, OC: ° F.                      | 355   | 20 |
| Pour: ° F.                          | 60    |    |
| Color, ASTM Union                   | 2.0   |    |
| Carbon Residue, Conradson: percent  | 0.02  |    |
| Copper Strip Test, 212° F., 3 hr.   | 0     |    |
| Neutralization Value ASTM D974-51T. |       | 25 |
| Total Acid No.                      | 0.05  |    |

#### EXAMPLE VI

Another composition is prepared by admixture of the cocoamine salt of dioctyl orthophosphoric acid to the oil-containing gasoline fuel composition of Example V. The cocoamine diisooctyl o-phosphate (84 weight percent oil concentrate) in this composition is added to the gasoline in the ratio of about 5 pounds per 1000 barrels (approximately 0.0019 percent by weight active component).

#### EXAMPLE VII

Another composition having excellent preignition characteristics is prepared in the manner of the foregoing Example I by incorporating in a gallon of the base gasoline 0.406 grams (0.1 theory) (approximately 0.014 weight percent) of molybdenum hexacarbonyl and 0.831 grams (0.2 theory) (approximately 0.029 weight percent) of tri(butoxyethyl)phosphate.

#### EXAMPLE VIII

Another composition is prepared in the manner of the foregoing Example I by incorporating in a gallon of the base gasoline 0.54 grams (0.1 theory) (approximately 0.019 weight percent) of tungsten hexacarbonyl and 0.831 grams (0.2 theory) (approximately 0.029 weight percent) of tri(butoxyethyl)phosphate.

#### EXAMPLE IX

Another satisfactory composition is prepared as indicated in Example VIII except that 0.27 grams (0.05 theory) of tungsten hexacarbonyl is used with 0.2 theory of tri(butoxyethyl)phosphate.

#### EXAMPLE X

Another satisfactory composition is prepared as indicated in Example VIII except that 0.135 grams (0.025 theory) of tungsten hexacarbonyl is used with 0.2 theory of tri(butoxyethyl)phosphate.

#### EXAMPLE XI

Another satisfactory composition is prepared as indicated in Example VIII except that 0.054 grams (0.01 theory) of tungsten hexacarbonyl is used with 0.2 theory of tri(butoxyethyl)phosphate.

#### EXAMPLE XII

Another satisfactory composition is prepared as indicated in Example VIII except that 0.276 grams (0.1 theory) of methyl diphenyl phosphate is used with 0.1 theory of tungsten hexacarbonyl.

An appreciable reduction in preignition due to tetraethyl lead decomposition product deposits is achieved by the use of the foregoing gasoline fuel compositions in internal combustion engines of the gasoline-powered, spark ignition type. For example, when the compositions described in the examples are burned in an internal combustion engine operated under conditions wherein noise, including preignition, knock or rumble would normally be encountered such engine noise is markedly less than the noise encountered when the base gasoline is used alone.

In order to illustrate the improved preignition characteristics obtained with a fuel of the invention as determined by the wild ping count, the base gasoline was compared with compositions of the invention in a single cylinder CFR engine having a 7 to 1 compression ratio. The engine installation used was a modification of the standard ASTM assembly as described in the laboratory knock-rating test procedure CRC designation F-1-545 and CRC designation F-2-545. These tests are described in the CRC Handbook, 1946 edition, compiled by the Coordinating Research Council, Incorporated. The engine assembly was modified to the extent that the Waukesha CFR engine was equipped with an L-head cylinder instead of an overhead valve.

The engine was operated on a cycling schedule alternating between the following conditions:

|                              |       |       |
|------------------------------|-------|-------|
| Duration, seconds            | 50    | 150   |
| Speed, r.p.m.                | 600   | 900   |
| Load                         | None  | Full  |
| Air Fuel Ratio               | 13:1  | 11:1  |
| Ignition Timing              | 1 TDC | 1 TDC |
| Coolant Temperature, ° F.    | 148+3 | 148+3 |
| Oil Temperature, ° F.        | 160+5 | 160+5 |
| Carburetor, Intake Air, ° F. | 110+5 | 110+5 |
| Humidity Control             | (2)   | (2)   |

1 TDC—Top Dead Center.

2 Ice Tower.

Over the entire test, a period of about 6 days, a record is kept of the total number of wild pings encountered. The total number of wild pings encountered during the test period is indicative of preignition tendencies. To determine the total number of wild pings, the engine is equipped with an ionization gap and an electronic wild ping counter which records the total number of wild pings encountered during the test period. Control tests are made periodically inasmuch as the engine requirements have a tendency to change as the engine becomes older. The test results obtained in the single-cylinder CFR engine are set forth in Table I.

TABLE I

| Test No. | Composition                                                                        | Wild Ping Count |
|----------|------------------------------------------------------------------------------------|-----------------|
| 192      | Base Gasoline                                                                      | 7,354           |
| 194      | Base Gasoline plus 0.2 theory of molybdenum hexacarbonyl (Example I composition)   | 1,045           |
| 195      | Base Gasoline                                                                      | 6,402           |
| 196      | Base Gasoline plus 0.1 theory of molybdenum hexacarbonyl (Example III composition) | 410             |
| 199      | Base Gasoline                                                                      | 1,382           |
| 200      | Base Gasoline plus 0.05 theory of molybdenum hexacarbonyl (Example IV composition) | 703             |

The data in the foregoing Table I clearly indicate the improvement obtained in a single-cylinder engine having a compression ratio of 7 to 1 when a small amount of molybdenum hexacarbonyl is added to the base gasoline.

Additional single-cylinder tests were made using a commercial engine having a compression ratio of 9 to 1. The results of these tests are set forth in Table II.

TABLE II

| Test No. | Composition                                                                      | Wild Ping Count |
|----------|----------------------------------------------------------------------------------|-----------------|
| 21       | Base Gasoline                                                                    | 13,353          |
| 22       | Base Gasoline plus 0.2 theory of molybdenum hexacarbonyl (Example I composition) | 3,682           |
| 19       | Base Gasoline plus 0.2 theory of tungsten hexacarbonyl (Example II composition)  | 2,599           |

The data in the foregoing Table II clearly indicate the improvement obtained in a single-cylinder engine having a compression ratio of 9 to 1 when a small amount of molybdenum or tungsten hexacarbonyl is added to the base gasoline.

In order to illustrate still further the improved engine operating characteristics obtained with fuels of the invention, a test was employed in which the fuel was burned in commercially available multicylinder spark-ignition engines having compression ratios of 10 to 1 and 10.5 to 1. In this test, the engines are operated on a cycling schedule consisting of three minutes at 1500 r.p.m. at a 15 brake horsepower load, followed by a one-minute idle at 450 r.p.m. The spark advance is the manufacturers' setting. The coolant temperatures in and out are 150° ( $\pm 5^\circ$ ) and 160° F. ( $\pm 5^\circ$ ), respectively. The oil temperature is 180° F. ( $\pm 5^\circ$ ). At the end of each twenty-four hours under the above-described cycling schedule, noise requirement determinations are made. After the noise requirement determinations are made, the engines are then put back on the cycling schedule for another twenty-four hours. The cycling and noise requirement tests are continued for nine 24-hour periods or less if an equilibrium octane number requirement appears to have been reached.

The noise requirement determinations are made according to three successive steps. If noise is encountered in step one, then steps two and three are omitted. If noise is encountered in step two, the only step three is omitted. Noise in this test is intended to include preignition, normal knocking or rumble. The three successive steps of the test are as follows:

(1) At a speed of 1100 r.p.m. the throttle is opened to detent (that is, the rear barrels of the carburetor are just open) at 1-inch Hg intake manifold vacuum.

(2) The engine speed is increased to 1300 r.p.m. at 3-inch vacuum.

(3) The engine is accelerated at 10-inch vacuum from 1300 to 2000 r.p.m., standard spark, and held at this setting for 3 seconds (throttle wide-open at end of 3-second period).

Aural observations are made at steps (1), (2) and (3) and preignition, rumble and knock are recorded.

Ratings are made on the tank fuel (99 research octane number) and the actual noise requirement determined by the use of a set of commercial reference fuels up to an octane number of 113.5. For noise requirements in the range 113.5 to 120, leaded isoctane is used. Octane numbers above 100 are expressed in the approved extension scale, Wiese octane numbers, which are:

Performance No. 100 +100  
3

The data set forth in Table III summarize the average octane number required to prevent engine noise, including preignition, normal knocking and rumble, when the test engines were operated under the above test procedure with the base gasoline and the base gasoline containing molybdenum or tungsten hexacarbonyl and molybdenum or tungsten hexacarbonyl together with tri(butoxyethyl)-phosphate. Compositions prepared from the base gasoline containing 0.2 and 0.3 theory of tri(butoxyethyl)phosphate in the absence of molybdenum or tungsten hexacarbonyl are included for comparative purposes. The results of further tests on a fuel composition containing

an upper cylinder lubricant and a corrosion inhibitor are also shown.

5 TABLE III.—AVERAGE OCTANE NUMBER REQUIREMENT TO PREVENT ENGINE NOISE

| 10 | Fuel Composition                                                                                                                                                                                                                 | Engine |       |
|----|----------------------------------------------------------------------------------------------------------------------------------------------------------------------------------------------------------------------------------|--------|-------|
|    |                                                                                                                                                                                                                                  | A      | B     |
| 15 | Base Gasoline                                                                                                                                                                                                                    | 120+   | 120+  |
|    | Base Gasoline plus 0.1 theory of tungsten hexacarbonyl                                                                                                                                                                           | -----  | 120+  |
|    | Base Gasoline plus 0.2 theory of tri(butoxyethyl)phosphate                                                                                                                                                                       | -----  | 116+  |
|    | Base Gasoline plus 0.3 theory of tri(butoxyethyl)phosphate                                                                                                                                                                       | -----  | 115+  |
|    | Base Gasoline plus 0.2 theory of molybdenum hexacarbonyl (Example I composition)                                                                                                                                                 | -----  | 117   |
|    | Base Gasoline plus 0.2 theory of tungsten hexacarbonyl (Example II composition)                                                                                                                                                  | -----  | 104   |
| 20 | Base Gasoline plus 0.1 theory of molybdenum hexacarbonyl and 0.2 theory of tri(butoxyethyl)phosphate (Example VII composition)                                                                                                   | -----  | 114   |
|    | Base Gasoline plus 0.1 theory of tungsten hexacarbonyl and 0.2 theory of tri(butoxyethyl)phosphate (Example VIII composition)                                                                                                    | -----  | 104   |
|    | Base Gasoline plus 0.05 theory of tungsten hexacarbonyl and 0.2 theory of tri(butoxyethyl)phosphate (Example IX composition)                                                                                                     | -----  | 101   |
| 25 | Base Gasoline plus 0.2 theory of molybdenum hexacarbonyl, 0.5 vol. Percent Coastal Lubricating Oil and 5 pounds per 1,000 barrels of gasoline of the cocaoamine salt of diisooctyl orthophosphoric acid (Example VI composition) | 116    | ----- |

30 Engine A 10:1 Compression Ratio  
Engine B 10.5:1 Compression Ratio

The data in the foregoing Table II clearly indicate the improvement obtained in multicylinder engines having compression ratios of 10 to 1 and 10.5 to 1 when a small amount of molybdenum or tungsten hexacarbonyl is added to a base gasoline alone or in combination with an organo-phosphorus compound. As indicated hereinabove, it is ordinarily preferred to use amounts of metal hexacarbonyl above about 0.1 theory unless the metal hexacarbonyl is used in combination with another ignition control agent. In this regard, it will be noted from the data in Table III that 0.1 theory of tungsten hexacarbonyl gave not noticeable improvement in engine noise. When the amount was increased to 0.2 theory, the octane number requirement dropped to 104. When 0.1 theory of tungsten hexacarbonyl was used in combination with 0.2 theory of tri(butoxyethyl)phosphate the octane number requirement was also reduced to 104. The latter result is surprising since the improvement obtained is more than the additive effect of the two agents taken alone. It is also surprising to note that still further improvement is obtained when only 0.05 theory of tungsten hexacarbonyl is used together with 0.2 theory of tri(butoxyethyl)phosphate.

Additional noise requirement data were obtained in single cylinder engines having a 9.5 to 1 compression ratio and multicylinder engines having a 10.5 to 1 compression ratio. In these determinations, leaded isoctane-benzene (LIB) ratings were obtained. The leaded isoctane-benzene rating, like the average octane number requirement to prevent engine noise, is also a rating of the fuel required to prevent engine noise, including preignition, normal knocking and rumble. The number signifying the LIB rating indicates the lowest percentage of isoctane in a leaded isoctane-benzene mixture that can be burned in the engine without inducing noise. Hence, a low LIB number indicates an effective preignition additive. In this test the isoctane and benzene each contain 3 cc. of tetraethyl lead per gallon. Inasmuch as there is little if any volume change on mixing benzene with isoctane, the mixture is also assumed to contain 3 cc. of tetraethyl lead per gallon. The leaded isoctane-benzene ratings are shown in Table

| Fuel Composition                                                                                                               | Leaded Isooctane-Benzene (LIB) rating |          |          |
|--------------------------------------------------------------------------------------------------------------------------------|---------------------------------------|----------|----------|
|                                                                                                                                | Engine A                              | Engine B | Engine C |
| Base Gasoline                                                                                                                  | 100+                                  | 100+     | 100+     |
| Base Gasoline plus 0.1 theory of tungsten hexacarbonyl                                                                         |                                       |          | 100+     |
| Base Gasoline plus 0.2 theory of tri(butoxyethyl) phosphate                                                                    | 55                                    | 68       | 99+      |
| Base Gasoline plus 0.3 theory of tri(butoxyethyl) phosphate                                                                    |                                       |          | 94+      |
| Base Gasoline plus 0.2 theory of tungsten hexacarbonyl (Example II composition)                                                |                                       |          | 66       |
| Base Gasoline plus 0.1 theory of tungsten hexacarbonyl and 0.2 theory of tri(butoxyethyl) phosphate (Example VIII composition) |                                       |          | 68       |
| Base Gasoline plus 0.05 theory of tungsten hexacarbonyl and 0.2 theory of tri(butoxyethyl) phosphate (Example IX composition)  |                                       | 28       | 65       |
| Base Gasoline plus 0.025 theory of tungsten hexacarbonyl and 0.2 theory of tri(butoxyethyl) phosphate (Example X composition)  | 16                                    | 50       | -----    |
| Base Gasoline plus 0.01 theory of tungsten hexacarbonyl and 0.2 theory of tri(butoxyethyl) phosphate (Example XI composition)  | 80                                    | -----    | -----    |
| Base Gasoline plus 0.2 theory of methyl diphenyl phosphate                                                                     |                                       | 62       | -----    |
| Base Gasoline plus 0.1 theory of tungsten hexacarbonyl and 0.1 theory of methyl diphenyl phosphate (Example XII composition)   |                                       | 44       | -----    |

Engine A and Engine B—Single cylinder engines having a 9.5 to 1 compression ratio.  
 Engine C—Multicylinder engine having a 10.5 to 1 compression ratio.

The single cylinder engines (Engines A and B) data in the foregoing Table IV clearly show the improvement obtained in the leaded isoctane-benzene rating when 0.025 to 0.1 theory of tungsten hexacarbonyl is admixed with 0.1 to 0.2 theory of an organo-phosphorus compound. It will be noted from the multicylinder engine (Engine C) data in Table IV that 0.1 theory of tungsten hexacarbonyl gave no noticeable improvement in the LIB number. When the amount was increased to 0.2 theory, the LIB number dropped to 66. When 0.1 theory of tungsten hexacarbonyl was used in combination with 0.2 theory of tri(butoxyethyl) phosphate the LIB number was 68. The latter result is surprising since the improvement obtained is more than the additive effect of using 0.1 theory and 0.2 theory of tungsten hexacarbonyl and tri(butoxyethyl) phosphate, respectively. It is also surprising to note from the multicylinder engine data that the LIB number of the base gasoline containing 0.2 theory of tri(butoxyethyl) phosphate was reduced from 99+ to 65 by the addition of only 0.05 theory of tungsten hexacarbonyl.

While my invention is described with reference to various specific examples and embodiments, it will be understood that the invention is not limited to such examples

and embodiments and may be variously practiced within the scope of the claims hereinafter made.

I claim:

1. A gasoline motor fuel comprising a major amount of gasoline containing tetraethyl lead in an amount sufficient to produce a gasoline fuel composition having a motor octane number of at least about 85 and a research octane number of at least about 95, said gasoline fuel composition upon combustion normally tending to form deposits which induce preignition of the gasoline in the combustion chamber of a spark ignition engine and a small amount, sufficient to substantially reduce such preignition, of tungsten hexacarbonyl.
2. A gasoline motor fuel comprising a major amount of gasoline containing tetraethyl lead in an amount sufficient to produce a gasoline fuel composition having a motor octane number of at least about 85 and a research octane number of at least about 95, said gasoline fuel composition upon combustion normally tending to form deposits which induce preignition of the gasoline in the combustion chamber of a spark ignition engine and a small amount, sufficient to substantially reduce such preignition of a synergistic mixture of an organo-phosphorous ignition control agent and tungsten hexacarbonyl.
3. A gasoline motor fuel comprising a major amount of gasoline containing tetraethyl lead in an amount sufficient to produce a gasoline fuel composition having a motor octane number of at least about 85 and a research octane number of at least about 95, between about 0.005 and about 0.3 theory of tungsten hexacarbonyl and between about 0.1 and about 0.5 theory of an organo-phosphorus ignition control agent.
4. A gasoline motor fuel comprising a major amount of gasoline containing tetraethyl lead in an amount sufficient to produce a gasoline fuel composition having a motor octane number of at least about 85 and a research octane number of at least about 95, between about 0.02 and about 0.1 theory of tungsten hexacarbonyl and between about 0.1 and about 0.2 theory of tri(butoxyethyl) phosphate.

#### References Cited

#### UNITED STATES PATENTS

|              |         |                   |       |
|--------------|---------|-------------------|-------|
| 1,779,061    | 10/1921 | Danner et al.     | 44—68 |
| 45 1,954,865 | 4/1934  | Danner            | 44—67 |
| 2,410,829    | 11/1946 | Luten             | 44—67 |
| 2,626,208    | 1/1953  | Brown             | 44—73 |
| 2,654,697    | 10/1953 | Andress et al.    | 44—58 |
| 50 2,818,416 | 12/1957 | Brown et al.      | 44—68 |
| 2,863,742    | 12/1958 | Cantrell et al.   | 44—58 |
| 2,897,068    | 7/1959  | Pellegrini et al. | 44—69 |
| 2,902,983    | 9/1959  | Patberg           | 44—67 |
| 2,982,627    | 5/1961  | Lauer et al.      | 44—67 |
| 3,240,576    | 3/1966  | Neu               | 44—69 |

55 DANIEL E. WYMAN, Primary Examiner.

Y. H. SMITH, Assistant Examiner.